

# UNITED STATES PATENT OFFICE.

EDOUARD HAMÉLIUS, OF MARSEILLE, FRANCE.

## METHOD OF FORMING SAND FOUNDRY-CORES AND SUBSTANCE FOR USE THEREIN.

1,308,524.

Specification of Letters Patent.

Patented July 1, 1919.

No Drawing.

Application filed November 26, 1918. Serial No. 264,252.

To all whom it may concern:

Be it known that I, EDOUARD HAMÉLIUS, a subject of the French Republic, residing at 55 Rue Curiol, Marseille, France, have invented new and useful Improvements in Methods of Forming Sand Foundry-Cores and Substance for Use Therein, of which the following is a specification.

Linseed oil is used in foundries for agglomerating white sand.

In order to give consistency to cores it is necessary to previously add various ingredients such as flour, resin, dextrin and the like, to the sand but in spite of such precautions the mixture obtained possesses only slight cohesion which prevents such cores thus molded in sand from being handled and prevents their safe removal from the mold box without causing deformation, more particularly when it is a question of recessed or grooved pieces of a certain size.

In order to facilitate the setting of the mixture it has been necessary to use linseed oil boiled in combination with flour but the cores thus obtained are hardly more consistent and do not resist high pressures and the cast metal penetrates therein through the interstices produced by reason of the combustion of the particles of flour.

This invention has for its object to obviate these disadvantages.

By this invention a carefully selected agglomerating liquid is intimately mixed with the sand by repeated siftings whereby each grain of sand is brought into contact with the air in order to facilitate the absorption

of oxygen, that is to say the fermentation of the liquid. After a few hours a mastic will be formed which fixes the grains of sand in a solid mass which is for this reason capable of being handled and transported.

For this purpose it suffices to introduce into the boiled linseed oil about four per cent. of litharge which forms by fermentation a mastic which, on the heating of the core after the evaporation of the excess of linseed oil, gives the agglomerated mass a considerable degree of hardness enabling any framing to be dispensed with and thus greatly facilitating the molding of the recessed or grooved parts of all dimensions while resisting during the casting the strongest pressures and the highest temperatures.

Having now particularly described and ascertained the nature of my said invention and in what manner the same is to be performed, I declare that what I claim is:

1. A mastic liquid for agglomerating white sand used for foundry cores composed by adding a small proportion of litharge to boiled linseed oil.

2. A method of making foundry sand cores consisting in repeatedly sifting the sand with an admixture of boiled linseed oil containing a small proportion of litharge.

In testimony whereof I have signed my name to this specification.

EDOUARD HAMÉLIUS.

Witnesses:

E. DUCASSON,  
JOHN TRACY.